

# UNITED STATES PATENT OFFICE.

SAM DYSON, OF ELLAND, AND JOHN GASKELL, OF LONDON, ENGLAND.

## PROCESS OF MAKING PETROLEUM PRODUCTS.

SPECIFICATION forming part of Letters Patent No. 683,735, dated October 1, 1901.

Application filed October 29, 1900. Serial No. 34,866. (No specimens.)

To all whom it may concern:

Be it known that we, SAM DYSON, residing at the Atlas Works, Elland, county of York, and JOHN GASKELL, residing at 122 Queen's 5 Gate, London, England, subjects of the Queen of Great Britain, have invented certain new and useful Improvements in the Manufacture of Saponaceous Products from Mineral Oils, of which the following is a clear and exact 10 specification.

Our invention consists of a process of making a saponaceous product hereinafter called "petroleum emulsion" which is suitable as a base or raw material for the manufacture of 15 all kinds of soap, also for lubricating and other industrial purposes, as hereinafter specified.

Many attempts have been made to produce saponaceous compounds containing more or 20 less mineral oil, such as hydrocarbons of the paraffin series; but in order to obtain a uniform and stable product it was found necessary either to incorporate foreign matter—such as carnauba-wax, boracic acid, or resin— 25 with the materials usually employed for the manufacture of soap or to restrict the quantity of hydrocarbons to about twenty per cent. If a larger quantity of mineral oil is employed, it will easily separate from the mixture in the 30 shape of globules.

We have found that a stable and uniform saponaceous compound which is easily miscible with any quantity of hot or cold water may be obtained by working within certain 35 limits of temperature, hereinafter described, and that if the said saponaceous compound is used as an intermediate product in the manufacture of soft soap a uniform and suitable soft soap containing upward of twenty-five 40 per cent. of mineral oil may be made in a very short time—about three hours. For example, to produce from petroleum by means of oleic acid an emulsion soluble in or miscible with water we add to one hundred pounds of petroleum at least ten pounds of oleic acid, preferably from twenty to twenty-five pounds, (according to the nature of the required product,) in a jacketed pan while agitating. We heat the mixture to a temperature ranging 45 between 120° and 140° Fahrenheit and gradually add caustic-potash solution of 40° Baumé at the rate of three-fourths of a pound to each

pound of oleic acid employed. This produces a uniform and transparent petroleum-jelly which is miscible with water and which may be used for the various purposes hereinafter described; but we find that a more perfect saponification is produced by diluting this jelly with from twenty to fifty per cent. of water, while maintaining the temperature and continuing the agitating, the result being to form a petroleum emulsion which is readily miscible with hot or cold water in any proportions and which can be more easily mixed with soft soaps or other saponaceous compounds than is the case with the petroleum-jelly described above.

The quantity of alkali used for the saponification may be varied according to the nature of the product required. For instance, 70 emulsions intended for the manufacture of insecticide, sheep-dip, lubricants, and similar products should be neutral, while for most kinds of soap an excess of alkali is beneficial.

The temperatures mentioned above have given the best results, although the emulsion can be formed at a temperature of about ten degrees higher or lower than the limit stated. Instead of petroleum, such as kerosene or 80 lamp oil, we may use other mineral oils, which are liquid at the temperature used in the process, whether such oils are derived from the distillation of petroleum, tar, bituminous shale, or from other sources. Instead of oleic acid or olein we may use stearic, palmitic, or other similar fatty acids, according to the nature of the product.

The petroleum emulsion and petroleum-jelly used, as described, may be used as a raw 90 material or intermediate product in the manufacture of soft or hard soap, sheep-wash, insecticide, lubricants, and varnish.

To produce bright and clear soft soap, we take eight hundred pounds of petroleum emulsion, add to it two hundred pounds of oleic acid or olein and from one hundred and fifty to two hundred pounds of caustic-potash solution of 30° Baumé, according to the strength of the soap required, and thoroughly mix the 100 said materials by means of a mechanical mixer until the caustic liquor has been absorbed. By subsequently raising the temperature to about 185° to 190° Fahrenheit a

bright product is at once obtained. The quantity of oleic acid may be varied according to the quality of soap required.

To produce hard soap, we take soap made from animal or vegetable fat by any of the known methods, place the same in a mixing-pan, and gradually mix with it a quantity of petroleum emulsion varying between twenty and fifty per cent. of the weight of the finished product by means of the ordinary crutching apparatus used in soap-works. This addition considerably reduces the cost of the soap and increases its cleansing and detergent properties, while it also gives to the soap antiseptic properties and makes it a powerful disinfectant.

As indicated above, the saponaceous emulsion obtained as described may be used also as a raw material or base in the manufacture of insecticide, sheep-dip, lubricants, and similar products.

It is not new to use petroleum-jelly for the manufacture of saponaceous products by mixing it with ordinary soap; but the product then obtained is deficient in cleansing properties, because ordinary petroleum-jelly, known under the name of "vaseline," consists of heavy hydrocarbons, which will not dissolve grease or penetrate into textile fabrics or the skin-like benzin or other like mineral oils.

We make no general claim to the use of petroleum-jelly in the manner described above, but limit ourselves to emulsions or

jellies obtained by the saponification of fatty matter in mixture with mineral oils.

Having thus fully described our invention, what we claim as new, and desire to secure by Letters Patent, is—

1. The process of making petroleum emulsion, consisting in mixing mineral oil with fatty acid, heating the mixture uniformly between the temperature  $110^{\circ}$  to  $150^{\circ}$  Fahrenheit, gradually adding an alkaline solution and subsequently water, while constantly stirring, and maintaining the temperature, substantially as described.

2. The process of making soap, which consists in taking eight hundred parts of a petroleum emulsion consisting of petroleum, alkali and a fatty acid, adding thereto substantially two hundred parts of olein or oleic acid and one hundred and fifty to two hundred parts of caustic-potash solution of  $30^{\circ}$  Baumé and thoroughly mixing the said materials until the caustic liquor has been absorbed, substantially as described.

In witness whereof we have hereunto set our hands in the presence of two subscribing witnesses.

SAM DYSON.

JOHN GASKELL.

Witnesses to the signature of Sam Dyson:

DAVID J. BAILER,  
JOSH. H. THOMPSON.

Witnesses to the signature of John Gaskell:

J. WETTER,  
WALTER E. ROCHE.